

(No Model.)

E. FISCHER.

METHOD OF AND APPARATUS FOR MANUFACTURING ARTIFICIAL LEATHER.

No. 244,872.

Patented July 26, 1881.



WITNESSES:

*Paul Stark*  
*Otto Risch*



INVENTOR:

*Ewald Fischer*  
BY *Paul Goepf*  
ATTORNEY.

# UNITED STATES PATENT OFFICE.

EWALD FISCHER, OF KALTWASSER, NEAR WÜSTE-GIERSDORF, PRUSSIA,  
ASSIGNOR OF ONE-HALF TO M. E. COHN & WOLLPEIM, OF BERLIN,  
GERMANY.

## METHOD OF AND APPARATUS FOR MANUFACTURING ARTIFICIAL LEATHER.

SPECIFICATION forming part of Letters Patent No. 244,872, dated July 26, 1881.

Application filed February 5, 1881. (No model.)

*To all whom it may concern:*

Be it known that I, EWALD FISCHER, a resident of Kaltwasser, near Wüste-Giersdorf, in the Kingdom of Prussia, German Empire, have 5 invented Improvements in Methods of and Apparatus for Manufacturing Artificial Leather, of which the following is a specification.

This invention has reference to an improved method of and apparatus for the manufacture 10 of artificial leather which is insoluble in hot and cold water, capable of resisting even weak acids and bases, and which has the necessary pliability so as to be adapted for water-proof coverings, beltings, packings, hot and cold water 15 hose, and other applications in the trades.

The invention consists, essentially, in the successive treatment of the fabric which forms the base of my artificial leather, first, in baths or solutions which contain chromic salts, and 20 then in baths or solutions which contain glycerine and glue, by which treatment the imitation leather-surface is obtained. It is necessary that the different operations have to be performed in the dark, or at least in rooms 25 which are not exposed to direct light, the surfaces of leather being only exposed to the influence of direct light at the last stage in the process of manufacture, after the grain has been imparted thereto by pressure. The chemical 30 influence of the light has the effect to make the chrome-glue composition insoluble and to render the same water-proof. This is an essential point in the successful treatment of the fabric, as only in that case the intimate combination of all the 35 different compounds which are successively deposited upon the fabric can be obtained. If, for instance, after the surface has been exposed to the light, a second covering or layer of chrome-glue would be deposited upon the fabric 40 and again exposed to the light, the last layer would not assimilate or unite at all with the first layer, but would peel off. As the chrome-glue and the other compounds are deposited directly upon the fabric, a more intimate adhesion of the same to the fibers is obtained as 45 if the chrome-glue and other compounds are first mixed and then laid upon the fabric as has been done heretofore, in which case the peeling off, cracking, and blistering of the coat-

ing of chrome-glue is an inevitable result, destroying the appearance of the fabric and rendering it useless for practical purposes. 50

In the accompanying drawings, Figures 1, 2, and 3 represent sectional side elevations, and Fig. 4 a plan view, of an apparatus adapted 55 for manufacturing artificial leather according to my improved method.

Similar letters of reference indicate corresponding parts.

The different parts of the apparatus will be 60 described in connection with the treatment which the fabric receives until the same is finally completed.

The textile fabric *x*, which forms the body or base of my improved artificial leather, is first 65 passed through a tank, *a*, containing a solution or bath of one part of bichromate of potash ( $K_2Cr_2O_7$ ) in about forty-five parts of water of  $44^{\circ}$  centigrade. The fabric is drawn through the solution at a slow speed, so that 70 it is thoroughly impregnated by the chrome solution, while the superfluous solution is removed by means of two pressure-rolls, *b*, and returned over an inclined apron to the tank *a*. In place of the bichromate of potash any other 75 equivalent chrome-salt may be used, though bichromate of potash is to be preferred. Before the fabric is dry it is passed through a second tank, *c*, which is filled with a solution or bath consisting of one part of glue, one part 80 of glycerine, and six parts of water. In selecting glue for this purpose preference should be given to glue obtained from leather scraps and waste. The constituent parts of the second tank are thoroughly mixed before use by boiling them for two hours and keeping them by a steam-pipe at a temperature of  $75^{\circ}$  centigrade. The fabric is then again passed through the pressure-rolls *d*, which remove the superfluous glue solution. The fabric is then conducted 85 over guide-rolls at some distance from a metal plate, *e*, which latter is heated either by direct fire or by steam or hot gases, as desired. The heat radiated by the plate *e* evaporates the water of the glue and glycerine so- 90 lution and dries the fabric. 95

If artificial leather of greater thickness has to be manufactured, the fabric is passed through

a second and third glue and glycerine bath and again dried by a second drying-plate, *k*, as shown in the drawings. If necessary, a third and even fourth coating of glue and glycerine 5 may be laid upon the fabric.

To the solution which gives a second coat of glue and glycerine it is advantageous to add some antiseptic ingredients, such as salicylic acid or birch-tar, in the proportion of one part 10 of these ingredients to one hundred parts of the glue solution. It is furthermore advisable to add to two hundred parts of the glue-solution one and a half parts of poppy or linseed oil and two parts of turpentine, by which the 15 leather is fully protected against fermentation, and also adapted to be treated, after finishing, with fatty inks or blacking and dressing. The fabric is now passed through a tank, *f*, which contains a solution of one part of tannic acid 20 in twenty-five to thirty parts of water, by which a weak tanning of the glue is obtained, so that the mass deposited on the textile fabric is made capable of greater resistance. The fabric is then passed through the pressure-rolls *g*, then 25 through the second chrome-bath, *i*, which contains a solution of one part of bichromate of ammonia,  $(\text{NH}_4\text{Cr}_2\text{O}_7)$ , one part of ammonia, and one part of alcohol in twenty-five parts of water. This solution is kept at the low temperature of from  $10^{\circ}$  to  $11^{\circ}$  centigrade by a cooling-pipe, to prevent the dissolving of the layer 30 of glue. On leaving this solution the fabric is passed over a second drying-plate, *k*, and then drawn through the smoothing-rolls *l* and the 35 heating-rolls *m*, which are heated by steam or gas, and provided on their surface with the necessary grain or pattern which the leather has to receive. All these operations have to take place without exposing the fabric to direct light, though the fabric may be exposed 40 for a short time to light before it passes through the pattern-roll *m*. The fabric is now wound up and finally exposed to the influence of sun or daylight, or any other source of light the 45 rays of which are capable of producing the chemical changes in the chrome-glue. The exposure to light may last from one or more days up to six weeks, or more, according to the thickness of the fabric and the intensity of the light. 50 As the fabric in its passage through the different solutions is submerged into the same it is coated at both sides. For imitation leather, which is to be coated on one side only, the fabric, instead of being entirely submerged, is 55 simply passed flat over the surface of the baths.

In the manufacture of extra qualities of glossy leather it is necessary to employ large

glass plates, which are covered with a solution of one part of wax and fifty parts of benzine. For this quality of leather it is preferable to 60 add to the last bath about one per cent. of weakly-nitrated cellulose fibers, so as to give body to the same. Before the fabric is then laid on the glass plate the surface is moistened with a solution of twelve parts alcohol 65 and four parts sulphuric ether, which solution exerts a slight dissolving influence upon the fibers, and imparts to the surface a greater resistance.

By laying upon the surface of the fabric in 70 this manner successive coats of chrome-salts and glue and glycerine, and fixing finally these layers by exposure to light, so as to form a homogeneous coating, a fabric in imitation of leather is obtained which is far superior to that 75 obtained by the methods heretofore employed, in which a mixture of different ingredients is laid directly upon the fabric, which mixture, however, could never form the intimate and permanent union with the fabric by the practical applications of the article.

Having thus described my invention, I claim as new and desire to secure by Letters Patent—

1. The method herein described for producing artificial leather, consisting in first treating the fabric, under exclusion of direct light, with a solution of a suitable chrome-salt, then with one or more solutions of glue and glycerine, to one of which antiseptic and fatty substances are added, then with a solution of bichromate of ammonia, and finally, after the grain or pattern has been imparted to the surface, exposing the fabric to the action of the direct light, so as to render the chrome-glue layers insoluble, substantially as set forth. 95

2. As an improvement in apparatus for the successive treatment, in the absence of light, of fabrics in the manufacture of artificial leather, tanks and rolls attached thereto, in combination with pressure-rolls and heated plates or heated rolls, when used in the order shown and described, and for the purpose set forth. 100

3. The tanks *a c f i*, in combination with pressure-rolls *b d g l* and steam-heating rolls *m*, substantially as and for the purpose set 105 forth.

In testimony whereof I have signed my name to this specification in the presence of two subscribing witnesses.

EWALD FISCHER.

Witnesses:

BERTHOLD ROI,  
CARL FEHLERT.